

March 1, 1955

W. R. WHITE ET AL

2,703,284

SUBBING PHOTOGRAPHIC FILM

Filed Feb. 8, 1951



GALE F. NADEAU & WALTER R. WHITE  
Inventors

*Daniel J. Mayne*  
By

*Scranton C. Van Houten*  
Attorneys

2,703,284

## SUBBING PHOTOGRAPHIC FILM

Walter R. White and Gale F. Nadeau, Rochester, N. Y., assignors to Eastman Kodak Company, Rochester, N. Y., a corporation of New Jersey

Application February 8, 1951, Serial No. 210,055

5 Claims. (Cl. 95—9)

This invention relates to a method of subbing photographic film in which the polymerized mixture of a lower fatty acid ester of cellulose and an alkyl acrylate is employed as the subbing layer.

Various materials have been suggested as subbing agents in the making of photographic film. Some subbing agents which have been suggested have been poor in adhesiveness, others when in use exhibit brittle characteristics, others have shown properties characterized by a changing in position of the emulsion on photographic film with reference to the rest of the film, known as "skidding."

One object of our invention is to provide a method of subbing photographic film to contribute to the flexibility thereof. Another object of our invention is to provide a method of subbing photographic film in which any skidding of the layers therein is reduced to a minimum. A further object of our invention is to employ as a subbing layer for photographic film the polymerized mixture of a lower fatty acid ester of cellulose and an alkyl acrylate. Other objects of our invention will appear herein.

We have found that subbing layers essentially consisting of a polymerized mixture of a lower fatty acid ester of cellulose and an alkyl acrylate provide good adhesiveness, prevent skidding of the emulsion thereon, contribute to the flexibility of the film and are also readily adapted to use for subbing purposes.

The accompanying drawing illustrates an enlarged sectional view of a photographic film base containing a subbing layer according to our invention; the figure being the sectional view of a cellulose ester film base subbed with successive layers of (1) the polymerized mixture of a fatty acid ester of cellulose and an alkyl acrylate, (2) cellulose nitrate, and (3) gelatin. By applying a layer of the photographic emulsion thereon over the gelatin coating, there is obtained a completed photographic film.

The subbing layer, in accordance with our invention, may be prepared from a polymerized mixture in which has been used any of the lower fatty acid esters of cellulose such as cellulose tripropionate, cellulose acetate butyrate, cellulose acetate, or any of the esters of cellulose and a fatty acid of 2 to 4 carbon atoms. The alkyl acrylate used may be ethyl acrylate, methyl acrylate, methyl methacrylate, or the like.

A polymerized mixture of a lower fatty acid ester of cellulose and the alkyl acrylate is conveniently prepared in the following manner:

A slurry is prepared of the cellulose ester, in a very finely divided or powder form, in water using a wetting agent. There is then mixed therewith an emulsion of the alkyl acrylate in water together with an emulsifier, a catalyst, and any other modifying materials desired. These compositions may be prepared as follows:

|                                                                                                                                                          | Parts |
|----------------------------------------------------------------------------------------------------------------------------------------------------------|-------|
| 1. Alkyl acrylate                                                                                                                                        | 23    |
| Water                                                                                                                                                    | 48    |
| Acetyl peroxide                                                                                                                                          | 0.5   |
| A higher sodium alkyl sulfate, the alkyl being of the order of C <sub>14</sub> known as Tergitol penetrant No. 4 in the form of its 30% aqueous solution | 0.7   |
| Sodium bisulfite                                                                                                                                         | 11    |
| 2. Cellulose ester                                                                                                                                       | 10    |
| Water                                                                                                                                                    | 40    |
| Tergitol penetrant No. 4 in the form of its 30% aqueous solution                                                                                         | 0.2   |

After these two compositions have been thoroughly mixed, the mixture is polymerized by tumbling it at 55° C. for three (3) days. The product obtained is then filtered, washed, and dried. This product is soluble in acetone, ethylene chloride and other organic solvents.

A polymerized mixture of cellulose ester and alkyl acrylate may be obtained by dissolving the cellulose ester in the acrylate, preferably in the proportions of 20-40% of the cellulose ester and 80-60% of the acrylate. The solution thus obtained is then dispersed in a composition of water and an emulsifier. The emulsifier may be a material such as gum arabic, polyvinyl alcohol, or some other similar dispersing material, such that the acrylate containing the cellulose ester may be uniformly dispersed in the water. The acrylate solution is conveniently dispersed in water in the proportions of 3 parts of water to 1 part of the acrylate solution, although greater dilutions may be advantageously employed if desired. Also, incorporated in the mass is a small proportion of a peroxide catalyst such as benzoyl peroxide. The polymerization is carried out by employing an elevated temperature such as 60° to 80° C. for the time found desirable to give the necessary polymerization. Ordinarily, 24 hours is adequate although other times may be used such as within the range of 6-48 hours. There results in this polymerization beads which may be easily dispersed by dissolving in an organic solvent such as acetone, ethylene chloride, and the like, or their mixtures. If desired, additional cellulose ester may be added to the polymerized mixture used for the subbing layer.

The cellulose ester which is employed as the film base may be a hydrolyzed cellulose acetate, a substantially fully esterified cellulose acetate, ordinarily known as triacetate, or a mixed ester of cellulose, such as cellulose acetate propionate, or cellulose acetate butyrate, all as are known for film base purposes. A subbing layer as described herein may be applied directly to the film base and, if desired, a subbing layer of subbing-type cellulose nitrate may be applied thereover. There may then be applied a layer of photographic emulsion, but preferably a layer of gelatin is first applied followed by the application of a layer of photographic emulsion thereover. Instead of employing separate layers of cellulose nitrate and gelatin prior to applying the emulsion layer, the cellulose nitrate and the gelatin are conveniently mixed together and applied as one layer to the film having the subbing layer thereon in accordance with our invention. For instance, a composition of the following proportions may be employed in applying this layer:

|                                                                                  | Per cent |
|----------------------------------------------------------------------------------|----------|
| Gelatin                                                                          | 1.2      |
| Cellulose nitrate                                                                | 0.3      |
| CrCl <sub>3</sub> ·6H <sub>2</sub> O 1.5% of the weight of the gelatin employed. |          |
| 55. Water                                                                        | 5.0      |
| Acetone                                                                          | 65       |
| Methanol the balance of the composition.                                         |          |

The application of this material may be by any recognized means of applying thin layers to film base. The application of this coating may be by means of rollers, brushes, air-knife, blades, sprays, or by any similar method which will apply the subbing coating to the film base in the form of a thin uniform layer without adversely affecting its properties. Whereas, with some types of subbing layers when the sensitized photographic film is incubated at 90° C. for 10 minutes, the emulsion "skids" so that the edges of the emulsion and of the film base may be as much as .020 inch apart, we have found that by employing as the subbing layer a product in which the cellulose ester and the acrylate are mixed together prior to polymerization that a photographic film is obtained which exhibits no "skidding" properties. We have also found that such a film exhibits properties more advantageous than are obtained by using as the subbing layer a physical mixture of the polymerized acrylate and the cellulose ester. The product so-obtained when coated with the usual gelatino-silver halide emulsion is found to have good flexibility and free of any skidding characteristics.

The following examples illustrate our invention:

Example 1.—30 parts of cellulose tripropionate was

dissolved in 70 parts of monomeric ethyl acrylate and the resultant solution was dispersed in water with agitation in the proportion of 1 part of solution to 3 parts of water, said water also containing a small amount of gum arabic to assist in the dispersing operation. .05 part of benzoyl peroxide was also incorporated therein. The mass was polymerized by heating at 60° to 80° C. for 24 hours. The polymer was obtained in bead form and was known as resin A.

3% of resin A was formed into a solution using 58% ethylene chloride, 5.5% ethyl acetate, and 33.5% acetone. This solution was coated onto a film support of cellulose triacetate plasticized with triphenyl phosphate to form a subbing layer of resin A thereon. There was then applied a coating of a cellulose nitrate layer from a solution of 2.25% cellulose nitrate in methyl alcohol which contained 5% butyl alcohol. There was then applied thereover a thin layer of a solution containing 0.9% gelatin in a solvent consisting of 1% glacial acetic acid, 15% water, and the balance methyl alcohol. As a check, a sample of the film base was subbed with a mixture of gelatin and cellulose nitrate followed by a layer of gelatin but without the subbing layer as described herein. The two samples were then coated with a photographic emulsion and were tested. It was found that the sample with the subbing layer as described herein tolerated much greater creasing before breaking occurred than the sample without that subbing layer. Also, when the film was suddenly compressed between the fingers after heating in an oven at 90° C. for 10 minutes, that in the case of the film in accordance with our invention, even though the emulsion had cracked, the support remained intact, whereas with the other sample, complete breaking of both emulsion and support occurred. The flexibility of the film in accordance with our invention, using the subbing layer as described, is far superior to that of the film in which that layer is not used. Both samples were found to be satisfactory as regards skidding of the emulsion and as regards adherence of the emulsion to the film.

*Example 2.*—A resin as described in the preceding example was formed into a solution using 58% ethylene chloride, 5.5% ethyl acetate and 33.5% acetone and the solution was coated onto film support of plasticized cellulose triacetate. There was then applied thereto a thin coating of a mixture of gelatin and cellulose nitrate from a composition having the following proportions:

|                                      |                                          |
|--------------------------------------|------------------------------------------|
| Gelatin                              | 1.2%.                                    |
| Cellulose nitrate                    | 0.3%.                                    |
| CrCl <sub>3</sub> .6H <sub>2</sub> O | 1.5% of the weight of the 50<br>gelatin. |
| Water                                | 5.0%.                                    |
| Acetone                              | 65%.                                     |
| Methanol                             | the balance.                             |

After this layer had been applied and dried, the film so-subbed was then coated with a photographic emulsion

layer and dried. The photographic film thus prepared was tolerant of severe creasing before any breaking occurred and any breaking which did occur was of the emulsion layer.

5 We claim:

1. A photographic film comprising a support of a lower fatty acid ester of cellulose, a subbing layer thereon essentially consisting of the material which results from heating an aqueous dispersion of a mixture of 20-40% of a cellulose ester and 80-60% of an alkyl acrylate containing a peroxide catalyst, and a silver halide-gelatin photographic emulsion layer.
- 10 2. A photographic film comprising a support of cellulose triacetate, a subbing layer thereon essentially consisting of the material which results from heating an aqueous dispersion of a mixture of 20-40% of a lower fatty acid ester of cellulose and 80-60% of an alkyl acrylate containing a peroxide catalyst, and a silver halide-gelatin photographic emulsion.
- 15 20 3. A photographic film comprising a cellulose acetate support, a subbing layer thereon essentially consisting of the material which results from heating an aqueous dispersion of a mixture of 20-40% of cellulose tripropionate and 80-60% of ethyl acrylate containing a peroxide catalyst, and a silver halide-gelatin photographic emulsion layer.
- 25 4. A photographic film comprising a cellulose organic ester support and in order thereon a subbing layer essentially consisting of the material which results from heating an aqueous dispersion of a mixture of 20-40% of a lower fatty acid ester of cellulose and 80-60% of an alkyl acrylate containing a peroxide catalyst, a cellulose nitrate layer, a gelatin layer and a silver halide-gelatin photographic emulsion layer.
- 30 35 5. A photographic film comprising a cellulose organic ester support and in order thereon a subbing layer essentially consisting of the material which results from heating an aqueous dispersion of a mixture of 20-40% of a cellulose ester and 80-60% of an alkyl acrylate containing a peroxide catalyst, a layer of a mixture of gelatin and cellulose nitrate and a silver halide-gelatin photographic emulsion layer.

References Cited in the file of this patent

UNITED STATES PATENTS

|           |                    |               |
|-----------|--------------------|---------------|
| 1,933,052 | Fikentscher et al. | Oct. 31, 1933 |
| 2,110,496 | Babcock            | Mar. 8, 1938  |
| 2,171,765 | Rohm               | Sept. 5, 1939 |
| 2,186,454 | Gloor              | Jan. 9, 1940  |
| 2,196,775 | McNally            | Apr. 9, 1940  |
| 2,271,228 | Nadeau et al.      | Jan. 27, 1942 |
| 2,292,393 | Mitchell           | Aug. 11, 1942 |

FOREIGN PATENTS

|         |               |               |
|---------|---------------|---------------|
| 487,795 | Great Britain | June 24, 1938 |
|---------|---------------|---------------|